

## UNITED STATES PATENT OFFICE

OTTO KAMPS, OF BERLIN, GERMANY

## ALUMINIUM ALLOY

No Drawing. Application filed May 8, 1930, Serial No. 450,877, and in Germany March 3, 1930.

This invention relates to an aluminium alloy with a percentage of silver, or silver and copper, essentially characterized by a percentage of thallium.

- 5 The new alloy possesses, in comparison with the known aluminium alloys, a number of valuable properties and is especially distinguished by high proofness against tarnishing. The new alloy comprises preferably 10 an addition of vanadium or palladium, and for certain purposes a further addition of nickel. Aluminium nickel alloys have become known, which however do not have the additions of this new alloy and therefore do 15 not possess the valuable properties of the same.

A method of increasing the tarnishing proofness of the new alloy forms part of the invention. This method is characterized in 20 that the alloy, in liquid state, is submitted, at a temperature of approximately 750° C., to a refining and purification by strontium chloride. The strontium chloride is preferably added, after the liquid metal has been 25 left standing for about 5 to 10 minutes without being touched, in an aluminium cartridge at the bottom of the liquid metal, whereupon the bath is thoroughly stirred several times and each time is carefully skimmed.

30 The new alloy is extraordinarily proof against tarnishing and shows no inclination to become black, in contrast to pure silver alloys which, when used, become black. This inconvenience of the pure silver alloys excludes their use for numerous purposes. The new alloy can further be easily treated and is at least equal, and in many respects even superior, to the commonly used silver-copper-aluminium alloys as regards color, resistance and hardness. It is proof against tarnishing, for instance in sulphurous atmospheres, and superior in this respect to sterling silver and pure silver. The alloy can be 40 cast to the finest wall thicknesses, as sand-

45 casting, chill-casting and extrusion-casting, and then shows resistances, which are equal to those of brass in cast and rolled condition. The alloy possesses also extraordinary adaptability for heavy drawings and is suitable to 50 be used in the industries engaged in the pro-

duction of vessels of any kind, of articles of decoration and for lighting purposes. It possesses an extraordinarily uniformly fine crystalline structure. The semi-manufactured articles made of the alloy can be rolled out in any lengths and widths and they do not smear, when being worked up.

55 The composition of the new alloy is preferably as follows: copper 2 to 5% or nickel 0.2 to 0.8% or copper and nickel in a total quantity of about 2 to 5%, silver 0.2 to 1%, thallium 0.02 to 0.2%, vanadium or palladium about 0.1%, the remainder commercial quality aluminium with the usual iron percentage 60 tolerances.

65 I claim:

1. A light metal alloy containing 0.2 to 1.0% of silver, and 0.02 to 0.2% of thallium, the remainder principally aluminium.

2. A light metal alloy containing 0.2 to 1.0% of silver, 2 to 5% of copper, and 0.02 to 0.2% of thallium, the remainder principally aluminium.

3. A light metal alloy containing 0.2 to 1.0% of silver, 2 to 5% of copper, 0.02 to 0.2% of thallium, and an appreciable amount of vanadium or palladium up to 0.1%, the remainder principally aluminium.

4. A light metal alloy containing 0.2 to 1.0% of silver, 2 to 5% of copper, 0.02 to 0.2% of thallium, and an appreciable amount of vanadium up to 0.1%, the remainder principally aluminium.

5. A light metal alloy containing 0.2 to 1.0% of silver, 2 to 5% of copper, 0.02 to 0.2% of thallium, an appreciable amount of vanadium up to 0.1%, and 0.2 to 0.8% of nickel, the remainder principally aluminium.

90 In testimony whereof I affix my signature.

OTTO KAMPS.

95

95

100